



US006159672A

# United States Patent [19]

Rieger et al.

[11] Patent Number: **6,159,672**[45] Date of Patent: **Dec. 12, 2000**

[54] **PHOTOGRAPHIC MATERIAL HAVING A BLUE SENSITIVE COUPLER STARVED UNIT**

5,190,851 3/1993 Chari et al. .... 430/506

[75] Inventors: **John Brian Rieger; James Anthony Friday**, both of Rochester, N.Y.

## FOREIGN PATENT DOCUMENTS

[73] Assignee: **Eastman Kodak Company**, Rochester, N.Y.

432834 6/1991 European Pat. Off. .  
1474994 5/1977 United Kingdom .  
91/06037 5/1991 WIPO .

[21] Appl. No.: **08/134,361**

[22] Filed: **Oct. 8, 1993**

*Primary Examiner*—Geraldine Letscher  
*Attorney, Agent, or Firm*—Arthur E. Kluegel

## Related U.S. Application Data

## ABSTRACT

[63] Continuation-in-part of application No. 08/003,178, Jan. 12, 1993, abandoned, which is a continuation of application No. 07/870,137, Apr. 16, 1992, abandoned.

The invention provides a multilayered color photographic element and associated image forming process wherein the element comprises a support having coated thereon photographic silver halide emulsion layers said layers including at least two blue sensitive layers, the blue sensitive layers being the emulsion layers farthest from the support, wherein the first of said blue sensitive layers is the most sensitive blue layer and is the emulsion layer farthest from the support, the first blue sensitive layer being extremely starved of dye-forming coupler, the second blue sensitive layer being contiguous said first blue sensitive layer.

[51] **Int. Cl.<sup>7</sup>** ..... **G03C 1/46**

[52] **U.S. Cl.** ..... **430/506**; 430/567; 430/503; 430/505; 430/957; 430/557; 430/555; 430/544; 430/558; 430/553

[58] **Field of Search** ..... 430/506, 567, 430/503, 505, 957, 557, 555, 544, 558, 553

## References Cited

**19 Claims, No Drawings**

## U.S. PATENT DOCUMENTS

2,376,217 5/1945 Wilder ..... 95/2

**PHOTOGRAPHIC MATERIAL HAVING A  
BLUE SENSITIVE COUPLER STARVED  
UNIT**

**CROSS-REFERENCE TO RELATED  
APPLICATIONS**

This application is a continuation-in-part of U.S. application Ser. No. 08/003,178 filed Jan. 12, 1993 now abandoned which is in turn a continuation of U.S. application Ser. No. 07/870,137 filed Apr. 16, 1992, now abandoned.

**BACKGROUND OF THE INVENTION**

This invention relates to a photographic material having multiple color layers comprising a unit of at least three green sensitive silver halide emulsion layers containing at least one magenta image dye-forming coupler which is also a bleach accelerating coupler.

Color photographic materials comprising multiple layers containing photographic couplers are well known. Typical photographic materials are described in U.S. Pat. Nos. 4,145,219; 4,724,198; 4,184,876; 4,186,016 and 4,724,198.

Prior photographic materials have exhibited problems with exposure reciprocity, speed, retained silver, color reproduction and neutral gray scale, flesh tone reproduction and image structure.

Various ways have been recognized in the photographic art for improving these problems. That is, for example, granularity can be improved but often it can be at the expense of another property such as speed. Or flesh tone color reproduction can be improved but neutral gray scale can be adversely affected. Thus, there is a great need for a photographic material which enables improvement in these properties without serious adverse affects.

U.S. Pat. No. 2,376,217 suggests that one way of avoiding the problems associated with the desensitization of emulsion layers due to the effects of the types of couplers in use in 1945 is to place a sensitized layer adjacent to the layer in question which is free of coupler. This will provide a layer which will not be adversely desensitized by the presence of coupler. The yellow couplers and the emulsions used today are not subject to desensitization problems, and thus, since this concern no longer exists, there would be no motivation to provide such a coupler-free layer in conjunction with today's couplers and emulsions.

**SUMMARY OF THE INVENTION**

The invention provides a multilayered color photographic element and associated image forming process wherein the element comprises a support having coated thereon photographic silver halide emulsion layers said layers including at least two blue sensitive layers, the blue sensitive layers being the emulsion layers farthest from the support, wherein

the first of said blue sensitive layers is the most sensitive blue layer and is the emulsion layer farthest from the support, the first blue sensitive layer being extremely starved of dye-forming coupler, the second blue sensitive layer being contiguous said first blue sensitive layer.

**DETAILED DESCRIPTION OF THE  
INVENTION**

The first green sensitive layer is suitably comprised of at least one magenta image dye-forming coupler (A), a timed development inhibitor releasing coupler, and preferably a

non-timed development inhibitor releasing coupler. The second layer is comprised of at least one first magenta image dye-forming coupler, (A), preferably at least one second magenta image dye-forming coupler, a development inhibitor releasing coupler and preferably a cyan dye-forming coupler. The third layer is comprised of at least one magenta image dye-forming coupler which is also a bleach accelerating releasing coupler. Further, the third layer contains a development inhibitor releasing coupler.

A typical photographic element in accordance with the invention comprises the following layer order:



The overcoat layer can be comprised of components known in the photographic art for overcoat layers including UV absorbers, matting agents, surfactants, and like. A UV layer can also be used which contains similar materials. UV absorbing dyes useful in this layer and the antihalation layer have the structure:



This layer, for example, also can contain dyes which can help in adjusting the photographic sensitivity of the element. Such dyes can be a green filter dye. A suitable green filter dye has the structure



A suitable red filter dye has the structure



Other dyes that may be used include washout dyes of the type referred to herein and filter dyes that decolorize during the photographic process.

#### Image Dye Forming Couplers

The image dye-forming couplers in the blue-sensitive, green-sensitive and red sensitive layers as described can be any of the image dye-forming couplers known in the photographic art for such layers for forming yellow, magenta and cyan dye images. Such couplers can comprise a coupler moiety (COUP) known in the art and as described. Combinations of the image dye-forming couplers can be useful in the described photographic silver halide emulsion layers.

Couplers that are yellow dye forming couplers are typically acylacetamides, such as benzoylacetanilides and pivalylacetanilides. Such couplers are described in such representative patents and publications as: U.S. Pat. Nos. 2,875,057; 2,407,210; 3,265,506; 2,298,443; 3,048,194; 4,022,620; 4,443,536; 3,447,928 and "Farbkuppler: Eine Literaturübersicht", published in Agfa Mitteilungen, Band III, pages 112-126 (1961).

The couplers that are cyan image dye-forming couplers (C) are typically phenols or naphthols, such as described in the photographic art for forming cyan dyes upon oxidative coupling.

Examples of such couplers (C) that form cyan dyes are typically phenols and naphthols that are described in such representative patents and publications as: U.S. Pat. Nos.

2,772,162; 3,772,002; 4,526,864; 4,500,635; 4,254,212; 4,296,200; 4,457,559; 2,895,826; 3,002,936; 3,002,836; 3,034,892; 2,474,293; 2,423,730; 2,367,531; 3,041,236; 4,443,536; 4,124,396; 4,775,616; 3,779,763; 4,333,999 and 5 "Farbkuppler: Eine Literaturübersicht", published in Agfa Mitteilungen, Band III, pages 156-175 (1961).

Examples of couplers (A) that form magenta dyes are typically pyrazolones, pyrazolotriazoles and benzimidazoles, such couplers are described in such representative patents and publications as U.S. Pat. Nos. 2,600,788; 2,369,489; 2,343,703; 2,311,082; 3,824,250; 3,615,502; 4,076,533; 3,152,896; 3,519,429; 3,062,653; 2,908,573; 4,540,654; 4,443,536; 3,935,015; 3,451,820; 4,080,211; 4,215,195; 4,518,687; 4,612,278; and European Applications 284,239; 284,240; 240,852; 177,765 and "Farbkuppler: Eine Literaturübersicht", published in Agfa Mitteilungen, Band III, pages 126-156 (1961).

The photographic element may be processed to form a developed image in an exposed color photographic element by developing the element with a color developer.

#### Fast Yellow

The fast yellow layer is a coupler starved layer exhibiting extreme coupler starvation. As used herein by coupler starved is meant a condition in the layer in which there is less dye-forming coupler than is theoretically capable of reacting with all of the oxidized developing agent generated at maximum exposure. Extreme coupler starvation is evidenced by a layer having a weight ratio of dye forming coupler to photographic silver halide (expressed as silver) of less than 0.10. In an embodiment of the invention, the weight ratio of dye-forming coupler to photographic silver halide (expressed as silver) is not more than 0.10. More suitably, the ratio is less than 0.05 and even more suitably less than 0.03. The layer is preferably substantially free of an image dye-forming coupler. The term dye-forming coupler means any coupler which will react with oxidized developer to form a yellow image dye. The coupler may be termed an "image dye-forming" coupler if the coupler does not contain a coupling-off group which has a photographic function. Couplers other than image dye-forming couplers can be present in this layer and such couplers can include, for example, timed development couplers as noted or non-timed DIR couplers and color correcting couplers. These other couplers are typically used at concentrations known in the photographic art and usually produce yellow dye typically not more than about 3% of the total density of the yellow record.

In the photographic element, the more blue sensitive layer or fast yellow layer contains a timed development inhibitor releasing coupler (DIR). Suitable timed DIR couplers used in the fast yellow layer comprise a DIR coupler (E) that is capable of releasing a mercapto-tetrazole development inhibitor comprising a substituent:



characterized in that

60 X is alkylene of 1 to 3 carbon atoms and R is alkyl of 1 to 4 carbon atoms, and the sum of the carbon atoms X and R is 5 or less. The DIR coupler is typically a pivalylacetanilide coupler, such as described in U.S. Pat. No. 4,782,012.

The timed DIR coupler can be any timed DIR coupler useful in the photographic art which will provide a timed development inhibitor release.

5

That is, a development inhibitor releasing coupler containing at least one timing group (T) that enables timing of release of the development inhibitor group can be any development inhibitor releasing coupler containing at least one timing group known in the photographic art. The development inhibitor releasing coupler containing at least one timing group is represented by the formula:



characterized in that

COUP is a coupler moiety, as described, typically a cyan, magenta or yellow dye-forming coupler moiety;

T and T<sup>1</sup> individually are timing groups, typically a timing group as described in U.S. Pat. Nos. 4,248,962 and 4,409,232;

n is 0 or 1; and

$Q^1$  is a releasable development inhibitor group known in the photographic art.  $Q^1$  can be selected from the INH group as described.

A preferred coupler of this type is described in U.S. Pat. No. 4,248,962.

Preferred timed DIR couplers of this type are:



6

Highly suitable timed DIR couplers have the structure:



Color from the fast yellow layer is produced mostly as a result of oxidized developer formed in the fast yellow layer migrating to the adjacent slow yellow layer and reacting to form yellow dye.

65 Other couplers that are development inhibitor releasing couplers as described include those described in for example U.S. Pat. Nos. 4,248,962; 3,227,554; 3,384,657; 3,615,506;

3,617,291; 3,733,201; and U.K. 1,450,479. Preferred development inhibitors are heterocyclic compounds, such as mercaptotetrazoles, mercaptotriazoles, mercaptooxadiazoles, selenotetrazoles, mercaptobenzothiazoles, selenobenzothiazoles, mercaptobenzoxazoles, selenobenzoxazoles, mercaptobenzimidazoles, selenobenzimidazoles, benzotriazoles, benzodiazoles and 1,2,4-triazoles, tetrazoles, and imidazoles.

5

10

## Slow Yellow Layer

In the photographic element, the less blue sensitive layer or slow yellow layer contains a yellow image dye-forming coupler. Such yellow image dye-forming coupler can be any yellow dye-forming coupler useful in the photographic art.

15

Couplers that are yellow image dye-forming couplers are typically acylacetamides, such as benzoylacetanilides and pivalylacetanilides, such as described in the photographic art for forming yellow dyes upon oxidative coupling.

20

25

The yellow dye-forming coupler in the slow yellow layer is typically a pivalylacetanilide coupler containing a hydantoin coupling-off group. Such a coupler is illustrated by the formula:

30



characterized in that

R<sup>2</sup> is chlorine, bromine or alkoxy;

R<sup>3</sup> is a ballast group, such as a sulfonamide or carboxamide ballast group; and

35

40

Z is a coupling-off group, preferably a hydantoin coupling-off group as described in U.S. Pat. No. 4,022,620.

Yellow dye-forming couplers suitable for the slow yellow or less sensitive blue layer are:

45

50

Timed or non-timed DIR couplers as noted with respect to the fast yellow layer may also be used in the slow yellow layer.



(6)

55

## Interlayer

In the photographic element a yellow filter layer is provided between the slow yellow and the fast magenta. This layer can comprise Carey Lea silver (CLS), bleach accelerating silver salts, any oxidized developer scavenger known in the photographic art, such as described in U.S. Pat. No. 4,923,787, and a dye to enable improved image sharpness or to tailor photographic sensitivity of the element. A preferred oxidized developer scavenger is:

-continued

(29)



(30)



A preferred yellow dye-forming coupler for the slow yellow layer has the structure:

(19)





Other oxidized developer scavenger useful in the invention include:



When finely divided silver such as Carey Lea silver is used in the yellow filter layer and the photographic element contains a BARC, then preferably an interlayer is provided between the yellow filter and any other layer that contains a dye forming coupler. If a bleach accelerating silver salt (BASS) is used, preferably in the yellow filter layer, then it is preferred to provide an interlayer to isolate the BASS containing layer from the remainder of the film. This interlayer may contain the oxidized developer scavenger noted above. Further, the interlayer may be contiguous with the yellow filter layer and may be disposed on both sides of the yellow filter layer. Representative bleach accelerating silver salts are disclosed in U.S. Pat. Nos. 4,865,965; 4,923,784; 4,163,669. The bleach accelerating silver salts can comprise silver salts of mercapto propionic acid.

BARC and BASS compounds may be used in combination in the element.

Other representative bleach accelerating silver salts which may be used in the interlayer are structurally shown as follows:

Instead of using finely divided silver in the yellow filter layer, filter dyes may be used. When filter dyes are used, then the interlayer contiguous or adjacent the yellow filter layer may be omitted. Oxidized developer scavenger as referred to above may be used in the yellow filter layer with the filter dye. Examples of filter dyes such as washout or decolorizing dyes useful in the present invention are described in U.S. Pat. No. 4,923,788 incorporated herein by reference. Such filter dyes have the formula:



characterized in that R is substituted or unsubstituted alkyl or aryl, X is an electron withdrawing group, R' is substituted or unsubstituted aryl or a substituted or unsubstituted aromatic heterocyclic nucleus, and L, L', and L" are each independently a substituted or unsubstituted methine group.

Preferred alkyl groups include alkyl of from 1 to 20 carbon atoms, including straight chain alkyls such as methyl, 45 ethyl, propyl, butyl, pentyl, decyl, dodecyl, and so on, branched alkyl groups such as isopropyl, isobutyl, t-butyl, and the like. These alkyl groups may be substituted with any of a number of known substituents, such as sulfo, sulfato, sulfonamide, amido, amino, carboxyl, halogen, alkoxy, 50 hydroxy, phenyl, and the like. The substituents may be located essentially anywhere on the alkyl group. The possible substituents are not limited to those exemplified, and one skilled in the art could easily choose from a number of substituted alkyl groups that would provide useful compounds according to the formula.

Preferred aryl groups for R include aryl of from 6 to 10 carbon atoms (e.g., phenyl, naphthyl), which may be substituted. Useful substituents for the aryl group include any of a number of known substituents for aryl groups, such as 60 sulfo, sulfato, sulfonamido (e.g., butane-sulfonamido), amido, amino, carboxyl, halogen, alkoxy, hydroxy, acyl, phenyl, alkyl, and the like.

The filter dyes may be used in combination with the finely divided silver.

65 It will be appreciated that permanent yellow filter dyes can be used instead of CLS or washout-filter dyes, such permanent dyes, for example, have structures:

(33)



A decolorizing microcrystalline dye useful in the invention has the structure:

(18) 35



#### Fast Magenta Layer

The most green sensitive layer or fast magenta layer 50 comprises a magenta image dye-forming coupler (A), a timed development inhibitor releasing coupler (DIR), preferably a non-timed DIR coupler and preferably a masking coupler.

The magenta image dye-forming coupler (A) can be any 55 image forming coupler dye useful in the photographic art.

A typical magenta image dye-forming coupler is a pyrazolotriazole. Suitable couplers that form magenta dyes include:



**13**

-continued



(14)

**14**

-continued

A preferred magenta image dye-forming coupler has the structure:

15



(15)

25 Suitable timed DIR couplers comprise a DIR coupler (E) that is capable of releasing a mercaptotetrazole development inhibitor as noted with respect to the fast yellow layer.

30 The masking coupler can be any masking coupler suitable for use in a photographic element. Preferably the masking coupler has structure:



(35)

or



(36)

45



(22)

50

55

60

65

65

## 15

The masking coupler can be placed in any of the three magenta imaging layers.

The non-timed DIR coupler (B) used in the fast magenta layer can be any non-timed DIR coupler known in the photographic art. Examples of such non-timed DIR couplers are disclosed in U.S. Pat. No. 3,227,554 incorporated herein by reference.

Preferred non-timed DIR couplers (B) have the structure:



## Mid Magenta Layer

The mid-magenta or mid green sensitive layer comprises at least one first magenta image dye-forming coupler, and preferably at least one second magenta image dye-forming coupler, preferably a non-timed DIR coupler and preferably a cyan dye-forming coupler (C).

The first magenta image dye-forming coupler can be coupler (A) referred to in the fast magenta layer.

The second magenta image dye-forming coupler can be any image forming coupler dye useful in the photographic art and can include the magenta image dye-forming coupler (A) referred to in the fast magenta layer.

A typical magenta image dye-forming coupler is a pyrazolotriazole. A preferred second image dye-forming coupler is coupler (34).

Coupler (14) is another preferred second magenta image dye forming coupler.

Suitable non-timed DIR couplers useful in the mid magenta layer are as described for the fast magenta layer and can be preferred coupler (B), for example.

The described cyan image dye-forming coupler (C) can be any cyan image dye-forming coupler known in the photographic art with its use in the magenta record herein referred to as a color correcting coupler. The cyan image dye-forming coupler is typically a phenol or naphthol coupler described in such representative patents and publications as noted herein.

## 16

Preferred cyan image dye-forming couplers (C) for the mid magenta layer have the structures:



Coupler (21) may also be used in the mid magenta layer.

## Slow Magenta Layer

The slow magenta layer contains at least one magenta image dye-forming coupler which is preferably a bleach accelerating releasing coupler (BARC). The slow magenta layer also contains a development inhibiting releasing coupler (DIR) preferably a non-timed DIR.

The bleach accelerator releasing coupler can be any bleach accelerator releasing coupler known in the photographic art. Combinations of such couplers are also useful. The bleach accelerator releasing coupler can be represented by the formula:



characterized in that

COUP is a coupler moiety as described, typically a cyan, magenta or yellow dye-forming coupler moiety;  $\text{T}^2$  is a timing group known in the photographic art, typically a timing group as described in U.S. Pat. Nos. 4,248,962 and 4,409,323, the disclosures of which are incorporated herein by reference;

$m$  is 0 or 1;

$\text{R}^3$  is an alkylene group, especially a branched or straight chain alkylene group, containing 1 to 8 carbon atoms; and

$\text{R}^4$  is a water-solubilizing group, preferably a carboxy group.

## 17

Typical bleach accelerator releasing couplers are described in, for example, European Patent 193,389.

A suitable bleach accelerator releasing coupler has the structure:



A preferred bleach accelerator releasing coupler has the structure:



Combinations of bleach accelerating couplers may be used the bleach accelerating coupler can be used in the other imaging layer including the magenta imaging layers.

The DIR coupler for the slow magenta layer can be the same coupler (B) used for the fast magenta or mid magenta layer.

An interlayer may be added between the fast and mid or mid and slow magenta layers.

Cyan dye-forming coupler (C) may be used in the slow magenta layer as in the mid magenta layer.

## Interlayer

The interlayer between the slow magenta and the fast cyan layers can contain an oxidized developer scavenger or dyes that are added to adjust photographic speed or density of the film. A preferred oxidized developer scavenger is as described for the yellow filter layer. The dyes can be the same as for the UV layer and an additional dye which is useful in this layer can include coupler (11).

## Fast Cyan Layer

The fast cyan or most red sensitive layer contains a cyan image dye-forming coupler (C), a first non-timed DIR coupler, preferably a second non-timed DIR coupler, a masking coupler and a yellow image dye-forming correcting coupler.

The cyan image dye-forming coupler (C) useful in the fast cyan layer is as described for the mid magenta layer. The

## 18

preferred cyan image dye-forming coupler is the same preferred coupler (C) as for the mid magenta layer.

The first and second non-timed DIR couplers in the fast cyan layer or most red sensitive layer can be any development inhibitor releasing coupler known in the photographic art. Typical DIR couplers are described in, for example, U.S. Pat. Nos. 3,227,554; 3,384,657; 3,615,506; 3,617,291; 3,733,201 and U.K. 1,450,479. Such DIR couplers upon oxidative coupling preferably do not contain a group that times or delays release of the development inhibitor group. The DIR coupler is typically represented by the formula:

## COUP-INH

characterized in that COUP is a coupler moiety and INH is a releasable development inhibitor group that is bonded to the coupler moiety at a coupling position. The coupler moiety COUP can be any coupler moiety that is capable of releasing the INH group upon oxidative coupling.

The coupler moiety (COUP) is, for example, a cyan, magenta or yellow forming coupler known in the photographic art. The COUP can be ballasted with a ballast group known in the photographic art. The COUP can also be monomeric, or it can form part of a dimeric, oligomeric or polymeric coupler, in which case more than one inhibitor group can be contained in the DIR coupler.

The releasable development inhibitor group (INH) can be any development inhibitor group known in the photographic art. Illustrative INH groups are mercaptotetrazoles, selenotetrazoles, mercaptobenzothiazoles, selenobenzothiazoles, mercaptobenzimidazoles, selenobenzimidazoles, mercaptobenzoxazoles, selenobenzoxazoles, mercaptooxadiazoles, mercaptotiadiazoles, benzotriazoles, and benzodiazoles. Preferred inhibitor groups are mercaptotetrazoles and benzotriazoles. Particularly preferred inhibitor groups are described in for example U.S. Pat. Nos. 4,477,563 and 4,782,012.

Preferred DIR couplers within COUP-INH are coupler (37) and:



Timed DIR couplers which may be used in this layer have the structures of couplers (24), (27) and (28) and



The second non-timed DIR coupler which may be used in the fast cyan layer has the structure in



A further second non-timed DIR coupler which may be used in the fast cyan layer has the structure of coupler (37).

The masking coupler in the most red sensitive layer is typically a cyan dye-forming masking coupler, such as a naphthol cyan dye-forming masking coupler.

A preferred cyan dye-forming masking coupler for the cyan dye-forming layers of the photographic element is:



The yellow image dye-forming coupler can be any such coupler useful in the photographic art with its use in the cyan record sometimes referred to as a color correcting coupler. Couplers that are yellow dye forming couplers are typically

acylacetamides, such as benzoylacetanilides and pivalylacetanilides as noted. Such couplers are described in such representative patents and publications as noted earlier.

The yellow dye-forming coupler is preferably a pivalylacetanilide comprising a phenoxy coupling off group. Such yellow dye-forming couplers have the same structures as used in the slow yellow layer and the preferred coupler is coupler (6).

#### Slow Cyan Layer

The slow cyan or less sensitive red layer contains a cyan image dye-forming coupler (C), a timed DIR coupler or development inhibitor anchimeric releasing coupler (DIAR), a non-timed DIR coupler, and a yellow image dye-forming correcting coupler.

The cyan image dye-forming coupler can be the same cyan image dye-forming coupler (C) as used in the fast cyan layer. Also, the yellow image dye-forming correcting coupler can be the same yellow image dye-forming coupler as used in the fast cyan layer.

An illustrative development inhibitor releasing coupler containing at least one timing group (T) that enables timing of release of the development inhibitor group preferably has the structure of coupler (5).

The non-timed DIR coupler can be the same as for the fast cyan layer.

#### Interlayer

An interlayer is provided between the slow cyan layer and the antihalation layer. The interlayer can contain an oxidized developer scavenger. A preferred oxidized developer scavenger is as described for the yellow filter layer. This interlayer solves a problem of increased fog resulting from interaction of bleach accelerating releasing coupler with silver in the antihalation layer. Thus, providing this interlayer between a BARC containing layer anywhere in the element and the antihalation layer so as to isolate the antihalation layer from layers containing dye-forming couplers, permits the advantageous use of a BARC for good silver bleaching without increasing fog or Dmin with respect to the antihalation layer, for example, while maintaining desired acutance.

#### Antihalation Layer

The antihalation layer can contain very fine gray or black silver filamentary or colloidal silver, e.g. CLS, and preferably a UV absorbing dyes, gelatin and colored dyes such as coupler (11) to provide density to the film.

While the antihalation layer has been described with respect to silver, other materials can be substituted for or used in conjunction with the silver. That is, instead of using finely divided silver in the antihalation layer, filter dyes such as washout-dyes or decolorizing dyes of the type referred to herein may be used. When filter dyes are used in the antihalation layer, the interlayer adjacent the antihalation layer may be omitted. Oxidized developer scavenger may be omitted from the antihalation layer when filter dyes are used. Examples of dyes which may be used in the antihalation layer are described in U.S. Pat. No. 4,923,788 as noted earlier.

Bleach accelerating silver salts as described with respect to the yellow filter layer may be used in the antihalation layer in conjunction with the finely divided silver. When bleach accelerating silver salts are used in antihalation it is preferred to use the interlayer over the antihalation layer as noted to minimize fog or Dmin.

In the following discussion of suitable materials for use in the emulsions and elements of this invention, reference will be made to *Research Disclosure*, December 1989, Item 308119, published by Kenneth Mason Publications, Ltd., Dudley Annex, 12a North Street, Emsworth, Hampshire. P010 7DQ, ENGLAND, the disclosures of which are incorporated herein by reference. This publication will be identified hereafter by the term "Research Disclosure".

The silver halide emulsions employed in the elements of this invention can be negative-working. Suitable emulsions and their preparation are described in Research Disclosure Sections I and II and the publications cited therein. Suitable vehicles for the emulsion layers and other layers of elements of this invention are described in Research Disclosure Section IX and the publications cited therein.

In addition to the couplers generally described above, the elements of the invention can include additional couplers as described in Research Disclosure Section VII, paragraphs D, E, F and G and the publications cited therein. These couplers can be incorporated in the elements and emulsions as described in Research Disclosure Section VII, paragraph C and the publications cited therein.

The photographic elements of this invention or individual layers thereof, can contain brighteners (see Research Disclosure Section V), antifoggants and stabilizers (See Research Disclosure Section VI), antistain agents and image dye stabilizers (see Research Disclosure Section VII, paragraphs I and J), light absorbing and scattering materials (see Research Disclosure Section VIII), hardeners (see Research Disclosure Section IX), plasticizers and lubricants (See Research Disclosure Section XII), antistatic agents (see Research Disclosure Section XIII), matting agents (see Research Disclosure Section XVI) development modifiers (see Research Disclosure Section XXI) surfactants and coating aids.

The photographic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the element with a color developing agent to reduce developable silver halide and oxidize the color developing agent. Oxidized color developing agent in turn reacts with the coupler to yield a dye.

With negative working silver halide, the processing step described above gives a negative image.

Development is followed by the conventional steps of bleaching, fixing, or bleach-fixing, to remove silver and silver halide, washing and drying.

#### EXAMPLE I

A three color photographic film was prepared as follows using conventional surfactants, antifoggants and the materials indicated. After providing a developable image and then processing in accordance with the Kodak C-41 process (British Journal of Photographic, pp. 196-198 (1988)) excellent results e.g. improved color, sharpness, granularity and neutral scale, were obtained and manufacturing cost savings were realized. All silver halide emulsions were stabilized with 1.75 gm 4-hydroxy-6-methyl-1,3,3a,7-tetraazaindene per mole of silver. All silver halide emulsions were sensitized with the appropriate spectral red, green and blue sensitizing dyes.

| Support                     | mg/m <sup>2</sup>                             | mg/ft <sup>2</sup>                          |                                                                                                                                                                                                                                                                                                                                                                                                                                                                                         |
|-----------------------------|-----------------------------------------------|---------------------------------------------|-----------------------------------------------------------------------------------------------------------------------------------------------------------------------------------------------------------------------------------------------------------------------------------------------------------------------------------------------------------------------------------------------------------------------------------------------------------------------------------------|
| <u>Layer 1</u>              |                                               |                                             |                                                                                                                                                                                                                                                                                                                                                                                                                                                                                         |
| Antihalation Layer          | 215<br>91<br>91<br>14.3<br>2422               | 20<br>8.5<br>8.5<br>13<br>225               | Black colloidal silver<br>UV absorbing dye<br>coupler (1)<br>UV absorbing dye<br>coupler (2)<br>Blue filter dye (11)<br>Gelatin                                                                                                                                                                                                                                                                                                                                                         |
| <u>Layer 2</u>              |                                               |                                             |                                                                                                                                                                                                                                                                                                                                                                                                                                                                                         |
| Interlayer                  | 54<br>861                                     | 5.0<br>80.0                                 | D-Ox scavenging<br>coupler (3)<br>Gelatin                                                                                                                                                                                                                                                                                                                                                                                                                                               |
| <u>Layer 3</u>              |                                               |                                             |                                                                                                                                                                                                                                                                                                                                                                                                                                                                                         |
| Least Red Sensitive Layer   | 915<br>1238<br>603<br>36<br>86<br>3078        | 85<br>115<br>56<br>3.3<br>8.0<br>286        | Red sensitized silver<br>iodobromide emulsion<br>(4.5% iodide, tabular<br>grains with average<br>grain diameter 1.1<br>micron and average<br>grain thickness 0.1<br>micron),<br>Red sensitized silver<br>iodobromide emulsion<br>(0.5% iodide, cubic<br>grains with average<br>edge length 0.21<br>microns)<br>Cyan dye forming image<br>coupler (4)<br>Cyan dye forming<br>development inhibitor<br>release (DIR) coupler<br>(5)<br>Yellow dye-forming<br>image coupler (6)<br>Gelatin |
| <u>Layer 4</u>              |                                               |                                             |                                                                                                                                                                                                                                                                                                                                                                                                                                                                                         |
| Most Red-Sensitive Layer    | 1291<br>54<br>32.3<br>50<br>11<br>2368<br>4.3 | 120<br>5.0<br>3<br>4.6<br>1.0<br>220<br>0.4 | Red sensitized silver<br>iodobromide emulsion<br>(3% iodide, octahedral<br>grains with average<br>grain diameter 0.90<br>micron)<br>Cyan dye-forming image<br>coupler (4)<br>Cyan dye-forming<br>masking coupler (7)<br>Cyan dye-forming DIR<br>coupler (9)<br>Yellow dye-forming<br>image coupler (6)<br>Gelatin<br>Cyan dye-forming DIR<br>coupler (8)                                                                                                                                |
| <u>Layer 5</u>              |                                               |                                             |                                                                                                                                                                                                                                                                                                                                                                                                                                                                                         |
| Interlayer                  | 129<br>861<br>11<br>49                        | 12<br>80<br>1<br>4                          | Oxidized development<br>scavenger coupler (3)<br>Gelatin<br>Green filter dye (10)<br>Blue filter dye (11)                                                                                                                                                                                                                                                                                                                                                                               |
| <u>Layer 6</u>              |                                               |                                             |                                                                                                                                                                                                                                                                                                                                                                                                                                                                                         |
| Least Green-Sensitive Layer | 124                                           | 15                                          | Green sensitized<br>silver iodobromide<br>emulsion (3% iodide,<br>tabular grains with<br>average grain diameter<br>0.8 micron, and<br>average grain<br>thickness 0.1 micron)                                                                                                                                                                                                                                                                                                            |

-continued

| Support                           | mg/m <sup>2</sup> | mg/ft <sup>2</sup> |                                                                                                                                                        |
|-----------------------------------|-------------------|--------------------|--------------------------------------------------------------------------------------------------------------------------------------------------------|
| <u>Layer 7</u>                    | 592               | 55.0               | Green sensitized silver iodobromide emulsion (0.5% iodide, tabular gains with average grain diameter 0.5 and average grain thickness 0.1 micron)       |
|                                   | 161               | 15.0               | Magenta dye-forming image coupler that releases a bleach accelerating fragment (12)                                                                    |
|                                   | 12                | 1.1                | Magenta dye-forming DIR coupler (13)                                                                                                                   |
|                                   | 1507              | 140                | Gelatin                                                                                                                                                |
|                                   |                   |                    |                                                                                                                                                        |
|                                   | 969               | 90.0               | Green sensitized silver iodobromide emulsion (3% iodide, tabular grains with average grain diameter 0.8 micron and average grain thickness 0.1 micron) |
|                                   | 75.0              | 7.0                | Magenta dye-forming image coupler (14)                                                                                                                 |
|                                   | 54.0              | 5.0                | Magenta dye-forming image coupler (15)                                                                                                                 |
|                                   | 9.0               | 0.8                | Magenta dye-forming DIR coupler (13)                                                                                                                   |
|                                   | 11.0              | 1.0                | Cyan dye forming, image coupler (4)                                                                                                                    |
| <u>Layer 8</u>                    | 1238              | 115.0              | Gelatin                                                                                                                                                |
|                                   | 753.0             | 70.0               | Green sensitized silver iodobromide emulsion (6% iodide, tabular grains with average grain diameter 1.0 micron and average grain thickness 0.1 micron) |
|                                   | 22.0              | 2.0                | Magenta dye-forming image coupler (15)                                                                                                                 |
|                                   | 13.0              | 1.2                | Magenta dye-forming DIR coupler (13)                                                                                                                   |
|                                   | 65.0              | 6.0                | Magenta dye-forming development masking coupler (16)                                                                                                   |
|                                   | 26.0              | 2.4                | Yellow dye-forming DIR coupler (17)                                                                                                                    |
|                                   | 969               | 90.0               | Gelatin                                                                                                                                                |
| <u>Layer 9</u>                    |                   |                    |                                                                                                                                                        |
|                                   | 75.0              | 7.0                | D-Ox scavenging coupler (3)                                                                                                                            |
|                                   | 194.0             | 18.0               | Developer bleachable yellow filter dye (18)                                                                                                            |
| <u>Layer 10</u>                   | 861.0             | 80.0               | Gelatin                                                                                                                                                |
|                                   |                   |                    |                                                                                                                                                        |
| <u>Least Blue-Sensitive Layer</u> | 215.0             | 20.0               | Blue sensitized silver iodobromide emulsion (6% iodide, octahedral grains with average grain diameter of 0.65 micron)                                  |
|                                   | 129.0             | 12.0               | Blue sensitized silver iodobromide emulsion (5% iodide, octahedral grains with average grain diameter of 0.40 micron)                                  |
|                                   | 258.0             | 24.0               | Blue sensitized silver iodobromide emulsion                                                                                                            |

-continued

| Support                   | mg/m <sup>2</sup> | mg/ft <sup>2</sup> |                                                                                                                      |
|---------------------------|-------------------|--------------------|----------------------------------------------------------------------------------------------------------------------|
| 5                         |                   |                    | (5% iodide, octahedral grains with average grain diameter of 0.23 micron)                                            |
| 10                        |                   |                    | 1100. 97.0 Yellow dye-forming image coupler (19)                                                                     |
| <u>Layer 11</u>           |                   |                    | Gelatin                                                                                                              |
| Most Blue-Sensitive Layer | 377.0             | 35.0               | Blue sensitized silver iodobromide emulsion (6% iodide, octahedral grains with average grain diameter of 1.0 micron) |
| 15                        |                   |                    | 11.0 1.0 Yellow dye-forming DIR coupler (17)                                                                         |
|                           |                   |                    | Gelatin                                                                                                              |
| 20                        |                   |                    | 1076 100.0                                                                                                           |
| <u>Layer 12</u>           |                   |                    | First Protective Layer                                                                                               |
|                           | 215.0             | 20.0               | Unsensitized silver bromide Lippman emulsion (0.04 microns)                                                          |
| 25                        |                   |                    | 108.0 10.0 UV absorbing dye (1)                                                                                      |
|                           |                   |                    | 129.0 12.0 UV absorbing dye (2)                                                                                      |
|                           |                   |                    | 753.0 70.0 Tricresyl phosphate                                                                                       |
|                           |                   |                    | 1345 125.0 Gelatin                                                                                                   |
|                           |                   |                    | 40 0.4 Green absorbing dye (10)                                                                                      |
|                           |                   |                    | 20 0.2 Red absorbing dye (20)                                                                                        |
| 30                        |                   |                    | <u>Layer 13</u>                                                                                                      |
|                           |                   |                    | Second Protective Layer                                                                                              |
|                           | 44.0              | 4.1                | Matte polyvinyltoluene beads                                                                                         |
|                           | 883.0             | 82.0               | Gelatin                                                                                                              |

35 The example will provide improvement in one or more photographic properties such as reciprocity, granularity, speed, retained silver, color reproduction and neutral gray scale, flesh tone reproduction and image structure and also 40 provides cost savings due to reduction in the coupler required.

## EXAMPLE II

A three color photographic film was prepared using 45 conventional surfactants, antifoggants, image couplers, development inhibitor releasing couplers, masking couplers, bleach accelerator releasing couplers, silver iodobromide emulsions, and sensitizing dyes. A conventional coating structure was also employed; i.e. overcoat/ultraviolet light 50 absorbing layer/blue light sensitive layer of the highest sensitivity/blue light sensitive layer of lowest sensitivity/blue light absorbing layer/green light sensitive layer of highest sensitivity/green light sensitive layer of lowest sensitivity/interlayer/red light sensitive layer of highest 55 sensitivity/red light sensitive layer of lowest sensitivity/antihalation layer/acetate support.

Levels of silver, gelatin, and coupler were varied in the most blue light sensitive layer, hereafter referred to as the "fast yellow" layer, and the least blue light sensitive, here- 60 after referred to as the "slow yellow" layer. It is known that increasing gelatin in the fast yellow layer will affect optical characteristics. As gelatin increases, optical scattering increases (The Theory of the Photographic Process, James, 4th edition, 598-607). Increasing gelatin in the fast yellow 65 layer will also affect development characteristics. Another name for this effect is "coupler borrowing", where oxidized developer created in the fast yellow layer wanders down and

reacts with coupler in the slow yellow layer. When coupler borrowing occurs, higher gamma results in the low exposure area of the sensitometric curve.

The following experiments illustrate the problem and several known solutions to high gamma resulting from coupler borrowing.

| Variation         | Weight % C/S | FY gel level (g/m <sup>2</sup> ) | FY Emulsion |
|-------------------|--------------|----------------------------------|-------------|
| EXP1A comparative | 38.8         | 1.03                             | EMUL1       |
| EXP1B comparative | 38.8         | 1.03                             | EMUL2       |
| EXP2A comparative | 35           | 0.65                             | EMUL3       |
| EXP2B comparative | 35           | 1.29                             | EMUL3       |
| EXP2C comparative | 35           | 1.94                             | EMUL3       |
| EXP3A comparative | 27.5         | 1.55                             | EMUL3       |
| EXP3B invention   | 7.5          | 1.55                             | EMUL3       |
| EXP4A comparative | 30           | 1.55                             | EMUL3       |
| EXP4B invention   | 10           | 1.55                             | EMUL3       |
| EXP4C invention   | 0            | 1.55                             | EMUL3       |

Terms in the table are defined as follows:

C/S=weight of Coupler coated per unit area divided by the weight of Silver coated per unit area contained in the blue light sensitive layer of highest sensitivity. 'Coupler' here refers to total image dye forming coupler plus image dye forming development inhibitor releasing coupler.

FY=blue light sensitive layer of highest sensitivity.

SY=blue light sensitive layer of lowest sensitivity.

EMUL1=an octahedral silver bromoiodide emulsion, with a grain diameter of 0.9 microns, containing 1.25% iodide in a core region and 1.75% iodide in a subsurface region.

EMUL2=a polydisperse silver bromoiodide emulsion of non-distinct morphology, with an average grain diameter of 0.9 microns, containing 6.3% bulk iodide, with a precipitation scheme incorporating a run salt with a thiocyanate digest.

EMUL3=an octahedral silver bromoiodide emulsion, with a grain diameter of 0.9 microns, containing 2.5% iodide in a core region and 3.5% iodide in a subsurface region.

The results from these experiments are summarized in the table which follows:

| Variation         | under gamma | granularity |
|-------------------|-------------|-------------|
| EXP1A comparative | 0.61        | 0.024       |
| EXP1B comparative | 0.73        | 0.019       |
| EXP2A comparative | 0.95        | 0.022       |
| EXP2B comparative | 0.79        | 0.019       |
| EXP2C comparative | 0.73        | 0.019       |
| EXP3A comparative | 0.69        | 0.019       |
| EXP3B invention   | 0.54        | 0.018       |
| EXP4A comparative | 0.77        | 0.018       |
| EXP4B invention   | 0.60        | 0.018       |
| EXP4C invention   | 0.59        | 0.018       |

Terms in the table are defined as follows:

under gamma=gamma in the under exposure region of the sensitometric curve, measured from a log exposure located 0.15 density above minimum density, to a log exposure which is 0.40 log exposure units more exposed.

The "aim" low gamma in all of these experiments was 0.55

granularity=average root mean square of density fluctuation measured with a 48  $\mu\text{m}$  aperture, measured from a log exposure located 0.40 log exposure units more exposed than 0.15 density above minimum density, to a log exposure which is 0.80 log exposure units more exposed than 0.15 density above minimum density.

The goal of this series of experiments was to obtain a film with aim gamma in the under exposure region of the curve ( $\text{gamma}=0.55$ ), while yielding acceptable granularity and minimizing the thickness of the coated structure in order to minimize optical degradation from light scatter.

From experiment 1 (EXP1A, EXP1B), it is evident that an emulsion which has inherently low gamma can be used to obtain lower gamma in the under exposure region of the sensitometric curve, but this will result in undesirable granularity. In this case, the run salt thiocyanate digest emulsion (EMUL1) yields lower gamma but granularity which is 26% higher than that obtained from the higher gamma core/shell octahedra.

From experiment 2 (EXP2A, EXP2B, EXP2C), it is evident that lower gamma in the under exposure region of the sensitometric curve can be obtained by incorporating higher levels of gelatin in the FY layer. This is due to a decrease of coupler borrowing from the SY layer to the FY layer. This also results in a thickening of the coating structure, which will result in increased optical degradation of light to underlying layers.

From experiment 3 (EXP3A, EXP3B), the technique of extreme coupler starvation is employed to obtain close to aim gamma in the under exposure portion of the sensitometric curve, while utilizing the low granularity core/shell emulsion, and maintaining constant coating thickness. This is done by utilizing coupler borrowed from the slow layer for imaging from the fast layer. The only way to do this and maintain low gamma, low granularity, and minimize optical scatter is to incorporate extreme coupler starvation.

From experiment 4 (EXP4A, EXP4B, EXP4C), the technique of extreme coupler starvation is employed to obtain closer to aim gamma in the under exposure portion of the sensitometric curve, while utilizing the low granularity core/shell emulsion, and maintaining constant coating thickness. This is done by utilizing coupler borrowed from the slow layer for imaging from the fast layer. The only way to do this and maintain low gamma, low granularity, and minimize optical scatter is to incorporate extreme coupler starvation.

The invention has been described in detail with particular reference to particular embodiments thereof, but it will be understood that variations and modifications can be effected within the spirit and scope of the invention.

What is claimed is:

1. A multilayered color photographic element comprising a support having coated thereon photographic silver halide emulsion layers said layers including at least two blue sensitive silver halide emulsion layers of different sensitivities, the blue sensitive layers being the emulsion layers farthest from the support, wherein the first of said blue sensitive layers is the most sensitive blue layer and is the emulsion layer farthest from the support, wherein the weight ratio of dye-forming coupler to photographic silver halide (expressed as silver) in the first blue sensitive layer is not more than 0.10, the second blue sensitive layer being contiguous said first blue sensitive layer and containing an acylacetamide yellow dye-forming coupler.
2. The element of claim 1 wherein the ratio is less than 0.05.
3. The element of claim 3 wherein the ratio is less than 0.03.
4. The element of claim 1 wherein the yellow dye-forming coupler is selected from the group consisting of benzoylacetanilides and pivaloylacetanilides.
5. The element in accordance with claim 1 wherein the most sensitive blue layer is substantially free of yellow dye-forming coupler.

6. A multilayered color photographic element comprising a support having coated thereon photographic silver halide emulsion layers, said layers including at least two green sensitive silver halide emulsion layers of different sensitivities and at least two blue sensitive silver halide emulsion layers of different sensitivities, the blue sensitive layers being the emulsion layers farthest from the support, the first of said blue sensitive layers is the most sensitive blue layer and is the emulsion layer farthest from the support, wherein the weight ratio of dye-forming coupler to photographic silver halide (expressed as silver) in the first blue sensitive layer is not more than 0.10, the second blue sensitive layer being contiguous said first blue sensitive layer and containing an acylacetamide yellow dye-forming coupler, the first blue sensitive layer comprised of a dispersing medium and silver bromoiodide that

- 15 a) is octahedral silver bromoiodide;
- b) has a grain size within the range of 0.45 to 1.2 microns;
- c) contains 1 to 12 mole percent iodide;
- d) has a core region (A) comprising 50% to 90% by weight of the silver bromoiodide, a surface region (B) and a subsurface region (C) between core region (A) and surface region (B); wherein
- (i) subsurface region (C) contains an iodide concentration higher than the iodide concentration of core region (A).

7. The element in accordance with claim 6 wherein the first blue sensitive layer is free of yellow image dye forming coupler.

8. The element in accordance with claim 6 wherein the first blue sensitive layer is substantially free of yellow image dye-forming coupler.

9. A multilayered color photographic element comprising a support having coated thereon photographic silver halide emulsion layers said layers including at least three green sensitive silver halide emulsion layers of different sensitivities and at least two blue sensitive silver halide emulsion layers of different sensitivities, the blue sensitive layers being the emulsion layers farthest from the support,

- 40 (i) the first of said green sensitive layers being the green sensitive layer farthest from the support, the second of said green sensitive layers being less green sensitive than the first green sensitive layer, the third of said green sensitive layers being the green sensitive layer closest to the support and being less green sensitive than said second green sensitive layer, the green sensitive layers being adjacent;
- (ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, the second blue sensitive layer being contiguous said first blue sensitive layer and containing an acylacetamide yellow dye-forming coupler, the first blue sensitive layer comprised of a dispersing medium and silver bromoiodide that
- a) is octahedral silver bromoiodide;
- b) has a grain size within the range of 0.45 to 1.2 microns;
- c) contains 1 to 12 mole percent iodide;
- d) has a core region (A) comprising 50% to 90% by weight of the silver bromoiodide, a surface region (B) and a subsurface region (C) between core region (A) and surface region (B); wherein
- (i) subsurface region (C) contains an iodide concentration higher than the iodide concentration of core region (A).

10. The element in accordance with claim 9 wherein the first blue sensitive layer is substantially free of yellow dye-forming coupler.

11. A multilayered color photographic element comprising a support having coated thereon photographic silver halide emulsion layers said layers including at least three green sensitive silver halide emulsion layers of different sensitivities and at least two blue sensitive silver halide emulsion layers of different sensitivities, the blue sensitive layers being the emulsion layers farthest from the support,

- (i) the first of said green sensitive layers being the green sensitive layer farthest from the support, the second of said green sensitive layers being less green sensitive than the first green sensitive layer, the third of said green sensitive layers being the green sensitive layer closest to the support and being less green sensitive than said second green sensitive layer, the green sensitive layers being adjacent,
- (ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, the second blue sensitive layer being contiguous said first blue sensitive layer and containing an acylacetamide yellow dye-forming coupler, characterized by
- the first blue sensitive layer comprised of
- a) a timed development inhibitor releasing coupler;
- the second blue sensitive layer comprised of
- b) a yellow image dye-forming coupler;
- the first of said green sensitive layers comprised of
- c) at least one magenta image dye-forming coupler;
- d) a timed development inhibitor releasing coupler;
- e) a non-timed development inhibitor releasing coupler;
- the second of said green sensitive layers comprised of
- f) a first magenta image dye-forming coupler;
- g) a second magenta image dye-forming coupler;
- h) a development inhibitor releasing coupler, and
- the third of said green sensitive layers comprised of
- j) at least one magenta dye-forming bleach accelerating releasing coupler, and
- k) a development inhibitor releasing coupler.

12. The photographic element in accordance with claim 11 wherein one of the green sensitive layers includes a cyan dye-forming coupler.

13. The photographic element in accordance with claim 11 wherein the photographic silver halide emulsion in the blue layer comprises a dispersing medium and silver bromoiodide that

- a) is octahedral silver bromoiodide;
- b) has a grain size within the range of 0.45 to 1.2 microns;
- c) contains 1 to 12 mole percent iodide;
- d) has a core region (A) comprising 50% to 90% by weight of the silver bromoiodide, a surface region (B) and a subsurface region (C) between core region (A) and surface region (B); wherein
- (i) subsurface region (C) contains an iodide concentration higher than the iodide concentration of core region (A).

14. The element in accordance with claim 11 wherein the most sensitive blue layer is substantially free of yellow image dye-forming coupler.

15. A multilayered color photographic element comprising a support having coated thereon photographic silver

29

halide emulsion layers said layers including at least three green sensitive silver halide emulsion layers of different sensitivities and at least two blue sensitive silver halide emulsion layers of different sensitivities, the blue sensitive layers being the emulsion layers farthest from the support, characterized by

(i) the first of said green sensitive layers being the green sensitive layer farthest from the support, the second of said green sensitive layers being less green sensitive than the first green sensitive layer, the third of said green sensitive layers being the green sensitive layer closest to the support and being less green sensitive than said second green sensitive layer, the green sensitive layers being adjacent,

(ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, the second blue sensitive layer being contiguous said first blue sensitive layer and containing an acylacetamide yellow dye-forming coupler.

16. A multilayered color photographic element comprising a support having coated thereon photographic silver halide emulsion layers said layers including at least three green sensitive silver halide emulsion layers of different sensitivities and at least two blue sensitive silver halide emulsion layers of different sensitivities, the blue sensitive layers being the emulsion layers farthest from the support, characterized by

(i) the first of said green sensitive layers being the green sensitive layer farthest from the support, the second of said green sensitive layers being less green sensitive than the first green sensitive layer, the third of said green sensitive layers being the green sensitive layer closest to the support and being less green sensitive than said second green sensitive layer, the green sensitive layers being adjacent,

(ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, and being free of yellow image dye-forming coupler the second blue sensitive layer being contiguous said first blue sensitive layer and containing an acylacetamide yellow dye-forming coupler,

the first blue sensitive layer comprised of

60

a) a timed development inhibitor releasing coupler having the structure

30



the second blue sensitive layer comprised of

b) a yellow image dye-forming coupler having the structure



the first of said green sensitive layers comprised of

c) a first magenta image dye-forming coupler having the structure



d) a time development inhibitor releasing coupler having the structure



e) a non-timed development inhibitor releasing coupler having the structure

65

31



32



and

i) a cyan dye-forming coupler having the structure

and the second green sensitive layer comprised of

f) a first magenta image dye-forming coupler having the structure



g) a second magenta image dye-forming coupler having the structure



h) a development inhibitor releasing coupler having the structure



30 the third green sensitive layer comprised of

j) at least one magenta dye-forming bleach accelerating releasing coupler having the structure



and

50 k) a development inhibitor releasing coupler having the structure



17. A multilayered color photographic element comprising a support having coated thereon photographic silver halide emulsion layers said layers including at least two red sensitive silver halide emulsion layers of different sensitivities, three green sensitive silver halide emulsion

layers of different sensitivities and at least two blue sensitive silver halide emulsion layers of different sensitivities, the blue sensitive layers being the emulsion layers farthest from the support and the red sensitive layers being closest to the support, characterized by

- (i) the first of said green sensitive layers being the green sensitive layer farthest from the support, the second of said green sensitive layers being less green sensitive than the first green sensitive layer, the third of said green sensitive layers being the green sensitive layer closest to the support and being less green sensitive than said second green sensitive layer, the green sensitive layers being adjacent, 5
  - (ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, and being free of yellow image dye-forming coupler the second blue sensitive layer being contiguous said first blue sensitive layer and containing an acylacetamide yellow dye-forming coupler, 10
  - (iii) the first of said red sensitive layers being the most red sensitive layer and being the red sensitive layer farthest from the support, 15
- the first blue sensitive layer comprised of
- a) a timed development inhibitor releasing coupler; 20
  - the second blue sensitive layer comprised of
  - b) a yellow image dye-forming coupler, 25
  - the first of said green sensitive layers comprised of
  - c) at least one magenta image dye-forming coupler;
  - d) a timed development inhibitor releasing coupler;
  - e) a non-timed development inhibitor releasing coupler; 30
  - the second of said green sensitive layers comprised of
  - f) a first magenta image dye-forming coupler;
  - g) a second magenta image dye-forming coupler;
  - h) a development inhibitor releasing coupler, and 35
  - i) a cyan image dye-forming coupler,
- the third of said green sensitive layers comprised of
- j) a magenta dye-forming bleach accelerating releasing coupler, and 40
  - k) a development inhibitor releasing coupler, 45
  - the first of said red sensitive layers comprised of
  - l) at least one cyan image dye-forming coupler;
  - m) at least one development inhibitor releasing coupler;
  - n) a masking coupler;
  - o) a yellow dye-forming coupler; 50
- the second of said red sensitive layers comprising
- p) a cyan image dye-forming coupler;
  - q) a timed development inhibitor releasing coupler and 55
  - r) a yellow dye-forming coupler.
- 18. A multilayered color photographic element comprising a support having coated thereon photographic silver halide emulsion layers said layers including at least two red sensitive silver halide emulsion layers of different sensitivities, three green sensitive silver halide emulsion layers of different sensitivities and at least two blue sensitive silver halide emulsion layers of different sensitivities, the blue sensitive layers being the emulsion layers farthest from the support and the red sensitive layers being closest to the support, characterized by**
- (i) the first of said green sensitive layers being the green sensitive layer farthest from the support, the second of 60

said green sensitive layers being less green sensitive than the first green sensitive layer, the third of said green sensitive layers being the green sensitive layer closest to the support and being less green sensitive than said second green sensitive layer, the green sensitive layers being adjacent,

- (ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, and being free of yellow image dye-forming coupler, the second blue sensitive layer being contiguous said first blue sensitive layer and containing an acylacetamide yellow dye-forming coupler,
  - (iii) the first of said red sensitive layers being the most red sensitive layer and being the red sensitive layer being farthest from the support,
- the first blue sensitive layer comprised of

- a) a timed development inhibitor releasing coupler having the structure



the second blue sensitive layer comprised of

- b) a yellow image dye-forming coupler having the structure



the first of said green sensitive layer comprised of

- c) at least one magenta image dye-forming coupler having the structure



- d) a timed development inhibitor releasing coupler having the structure

35



36

-continued



5 e) a non-timed development inhibitor releasing coupler having the structure



10 h) a development inhibitor releasing coupler having the structure



15 and

the second green sensitive layer comprised of

20 f) a first magenta image dye-forming coupler having the structure



25 g) a second magenta image dye-forming coupler having the structure



30 i) a cyan image dye-forming coupler having the structure



35 the third green sensitive layer comprised of

40 j) a magenta dye-forming bleach accelerating releasing coupler having the structure



45 and

50 k) a development inhibitor releasing coupler, having the structure

37



the first of said red sensitive layers comprising:

1) a cyan image dye-forming coupler having the structure



m) at least one first development inhibitor releasing coupler having the structure



n) at least one second development inhibitor releasing coupler having the structure



38

38



p) a yellow dye-forming coupler having the structure



the second of said red sensitive layers comprising

q) a cyan image dye-forming coupler having the structure



r) a timed development inhibitor releasing coupler selected from at least one of



and



s) a yellow image dye-forming coupler having the structure



19. A multilayered color photographic element comprising a support having coated thereon photographic silver halide emulsion layers said layers including at least two red sensitive silver halide emulsion layers of different sensitivities, three green sensitive silver halide emulsion layers of different sensitivities and two blue sensitive silver halide emulsion layers of different sensitivities, the second of said green sensitive layers being less green sensitive than

the first green sensitive layer, the third of said green sensitive layers being less green sensitive than said second green sensitive layer characterized by

- 5 (i) the first of said green sensitive layers being the green sensitive layer farthest from the support, the second of said green sensitive layers being less green sensitive than the first green sensitive layer, the third of said green sensitive layers being the green sensitive layer closest to the support and being less green sensitive than said second green sensitive layer, the green sensitive layers being adjacent,
- 10 (ii) the first of said blue sensitive layers being the most sensitive blue layer and being the emulsion layer farthest from the support, wherein the weight ratio of dye-forming coupler to photographic silver halide (expressed as silver) in the first blue sensitive layer is not more than 0.10, and being free of yellow image dye-forming coupler, the second blue sensitive layer being contiguous said first blue sensitive layer and containing an acylacetamide yellow dye-forming coupler,
- 15 (iii) the first of said red sensitive layers being the most red sensitive layer and being the red sensitive layer being farthest from the support, a second red sensitive layer being the least red sensitive layer
- 20 the layers being arranged on the support in the following sequence with
  - a) an antihalation layer,
  - 25 b) a first interlayer comprised of gelatin and containing an oxidized development scavenger,
  - c) a second red sensitive layer comprised of
    - (i) a cyan image dye-forming coupler
    - (ii) a timed development inhibitor releasing coupler and
    - (iii) yellow dye-forming coupler
  - d) a first red sensitive layer comprised of
    - (i) at least one cyan image dye-forming coupler
    - (ii) at least one development inhibitor releasing coupler
    - (iii) a masking coupler
    - (iv) a yellow dye-forming coupler,
  - e) a second interlayer comprised of gelatin and containing an oxidized development scavenger
  - f) a third green sensitive layer comprised of
    - (i) a magenta dye-forming bleach accelerating releasing coupler and
    - (ii) a development inhibitor releasing coupler,
  - 35 g) a second green sensitive layer comprised of
    - (i) a first magenta image dye-forming coupler,
    - (ii) a second magenta image dye-forming coupler,
    - (iii) a development inhibitor releasing coupler, and
    - (iv) a cyan image dye-forming coupler
  - 40 h) a first green sensitive layer comprised of
    - (i) at least one magenta image dye-forming coupler,
    - (ii) a timed development inhibitor releasing coupler,
    - (iii) a non-timed development inhibitor releasing coupler;
    - (iv) a masking coupler
  - i) a yellow filter layer,
  - j) a second blue sensitive layer comprised of a yellow image dye-forming coupler,
  - k) a first blue sensitive layer comprised of a timed development inhibitor releasing coupler, and
  - 45 l) an overcoat layer.

UNITED STATES PATENT AND TRADEMARK OFFICE  
**CERTIFICATE OF CORRECTION**

PATENT NO. : 6,159,672  
DATED : December 12, 2000  
INVENTOR(S) : John Brian Rieger, James Anthony Friday

Page 1 of 1

It is certified that error appears in the above-identified patent and that said Letters Patent is hereby corrected as shown below:

Column 27,

Line 26, Claim 7 is amended to read as follows:

7. The element in accordance with claim 6 wherein the first blue sensitive layer is free of yellow image dye forming coupler.

Signed and Sealed this

Sixth Day of November, 2001

Attest:

*Nicholas P. Godici*

Attesting Officer

NICHOLAS P. GODICI  
*Acting Director of the United States Patent and Trademark Office*